

Patented Dec. 25, 1934

1,985,675

Leather having a printed design thereon, characterized by the use of a liquid coating of cellulose or similar material, which is applied to the surface of the leather, and which is dried, and then the leather is printed, and the printed surface is dried, and then a second liquid coating of cellulose or similar material is applied to the printed surface, and the second liquid coating is dried, and the leather is then glazed, and the glazed leather is dried, and the leather is then ready for use.

# UNITED STATES PATENT OFFICE

1,985,675

## PRINTED LEATHER

Peter A. Blatz, Westover Hills, Del.

No Drawing. Application January 27, 1932,

Serial No. 589,315

3 Claims. (Cl. 91—67.9)

My invention relates to the manufacture of leather, and comprises an improved method of manufacturing printed leather, and more particularly relates to the manufacture of glazed 5 kid with an all over design printed thereon.

Leathers having a printed design thereon are desirable for many purposes such, for instance as the use of cow hides split or whole for covering furniture; and the use of glazed kid for the 10 uppers of shoes, or as linings for shoes. Heretofore it has not been common to print a design upon such leathers, a condition that was due to both the unsatisfactory results obtained and to the relatively high costs of applying a printed 15 effect to a surface such as that presented by a hide or skin.

One object of the present invention is to provide a novel method of making printed skins or 20 hides in which the cost of application of the process to the skin and the success of the application is such that the product will be readily salable on a commercial basis.

A more specific object of the invention is to provide a method of making printed skins in which 25 a color carrying medium may be readily and economically placed upon the surface of a tanned skin; the printed impression applied over such surface or ground color, and a protective coating placed over the printed impression.

30 Other objects of my invention will be apparent from the following specification and from the appended claims.

While it is possible to use the skins or hides of 35 various animals, my improved method or process will be described in connection with the application of a printed surface to skins of young goats, familiarly known as "kid", with the understanding that my improved process may be similarly applied to other leathers differing in 40 character and intended use.

In carrying out my improved method or process of manufacturing printed leather I use a completely tanned skin, chrome, or otherwise tanned; that is to say, a skin which might normally be used for the manufacture of shoes or otherwise employed without the performance of further finishing steps thereon, except the glazing step. Upon a skin in this condition I carry out the method or process hereinafter described, 45 and as a result of the proper carrying out of such method or process I produce smooth, firm skins with printed designs thereon.

The tanned skin to be subsequently printed 50 may be "whitened" or given a ground color of any desired shade or tone which serves as a back-

ground for the printed matter, in any usual and suitable fashion. In the case of white skins, a white pigment may be applied, or the skins may be initially white and of a character substantially like those produced in carrying out the 5 process set forth in Patent No. 1,334,216, dated March 16, 1920. Upon such white, or whitened, or other colored skins I apply a normally insoluble liquid coating of any suitable and desired type having or containing cellulose such, 10 for example, as a pyroxylin coating. This finish may be applied by an ordinary paint brush or swab, or by means of an air brush or spray gun; the means for applying the coating being immaterial so long as the entire surface of the skin 15 to be subsequently printed is evenly covered with the coating.

Upon completing the application of this coating of cellulosic material to the surface of the skins, they may be flattened in any suitable manner as, for instance, by pressing them between the hot plates of a hydraulic press, so that when removed for the printing step they present a smooth, flat surface. A surface is thus provided 20 that is readily adapted to receive a printed impression and to which the ink or other material 25 so applied will readily adhere.

Upon completion of the pressing operation the skins may be printed in any desired fashion 30 with any suitable design. I have found by experiment that an ink or paint suitable for this purpose is any pigment which may be suspended in or by a body of casein. Pigments ground in oil such as printers' ink may also be used. I have discovered that an ink of this character will 35 readily adhere to the cellulosic base coating and, in addition, such printing medium will form a suitable base for the reception of a covering coat or coats of cellulosic material.

After the skins have been printed the printed 40 surface is dried in any usual or suitable manner, and upon completion of the drying of the printed impression, a second coat of the cellulosic material is applied over the printed impression. This 45 second coating may be applied in exactly the same manner in which the first coating was applied, and such second coating completely covers the printed surface. This final coating serves as a means for protecting the printed surface and for protecting the skin from damage by the elements; being substantially water- and/or moisture-proof.

Upon drying the final cellulosic coating the 50 skins may be glazed in the usual manner, and after the glazing step they are ready for use in 55

the manufacture of shoes and other footwear or for other purposes.

Various modifications may be made in the above embodiment of my invention without departing 5 from the spirit and scope thereof as set forth in the following claims.

I claim:

1. The method of making printed leather which comprises completely tanning a skin to 10 produce leather, apply a liquid cellulosic color-holding base to the entire surface of the tanned skin, printing a design upon such cellulosic base with a pigment carried in a casein medium, drying such printed surface, applying a thin coating 15 of a cellulosic material over the printed surface, drying such cellulosic coating and thereafter finishing the surface of the skin by a glazing operation.
2. The method of making printed leather which 20 comprises completely tanning a skin to produce leather, white-coating the entire surface of said

leather, applying a liquid cellulosic coating over said white coating, drying said coating, printing a design over the cellulosic coating with a pigment carried in a casein medium, drying such printed surface, applying a thin coating of a cellulosic material over the printed surface, drying such cellulosic coating and thereafter finishing the surface of the skin by a glazing operation. 5

3. The method of making printed leather which comprises completely tanning a skin by a chrome 10 treatment to produce leather, applying a liquid cellulosic coating over the entire surface of the tanned skin, flattening the skins by subjecting them to heavy pressure between hot plates, printing a design over the cellulosic coating with a 15 casein-held pigment, drying such printed surface, applying a thin coating of cellulosic material over the printed surface, drying such cellulosic coating, and thereafter finishing the surface of the printed skin by a glazing operation. 15

PETER A. BLATZ.

20